

1

3,079,259

## CYAN COLOR FORMERS

Emil B. Rauch, Port Dickinson, and Charles R. Hance, Endwell, N.Y., assignors to General Aniline & Film Corporation, New York, N.Y., a corporation of Delaware  
No Drawing. Filed July 21, 1960, Ser. No. 44,268  
2 Claims. (Cl. 96—100)

This invention relates to color photography and the production of colored photographic images by color forming development. More particularly, it relates to cyan color-forming couplers and to silver halide photographic emulsions containing them.

It is known to produce colored photographic images wherein a color former or coupling component reacts with the development product of a primary aromatic amino developing agent. In processes of this type, the subtractive method of color formation is ordinarily employed with the result that the photographic images so obtained are composed of the subtractive primary colors, i.e., cyan, magenta and yellow. In the multi-layer color systems in use today, magenta dye images are usually produced from pyrazolone structures; the yellow dye images are derived from reactive ketomethylene compounds, whereas the cyan images are produced from phenolic substances such as phenols or naphthols. Photographic dye images as above described are formed in situ with the silver images which are subsequently removed or otherwise bleached to leave the pure dye images.

One of the major difficulties confronting color photography is to provide dyes possessing proper spectral photographic properties. Thus, in a colored photographic reproduction employing the subtractive color process three subtractively colored dye images are placed in overlapping registration. The function of the subtractively dyed images, which are yellow, magenta and cyan respectively, is to modulate white light. Expressed in another manner each of the three subtractively superimposed images absorbs the required amount of white light. When the three dyed images are viewed in white light and in perfect register, a colored reproduction representing the colored aspects of the original subject is thereby produced.

Ideally, each of the three subtractively colored layers should absorb one-third of the visible light spectrum, i.e., the yellow image should absorb blue, the magenta should absorb green and the cyan layer should absorb in the red portion of the spectrum. However, in actual practice this latter condition is approached but never achieved. Consequently, the search for color couplers capable of yielding on color development a truer subtractively dyed image continues.

As previously pointed out, cyan dye images are commonly derived from naphthol color formers. Structures which have shown promise in this connection are the anilides of 1-hydroxy-2-naphthoic acid containing an alkoxy group in the ortho position of the anilide portion of the molecule and being further provided with carboxy or sulfo solubilizing functions. The latter are preferably located ortho or para to the alkoxy group. The compounds disclosed in the prior art although yielding dye images possessing desirably high stability under conditions of excessive humidity proved to be too green when used in a reversal color material. On investigation, it was found that the excessive greenish hue was not so much due to the absorption in the red sensitive region of the spectrum, as to the rather excessive blue absorption of the dyes produced from these couplers. It was realized that an excellent naphthol cyan color coupler might be evolved if it were possible to design a chemical structure having all the stability towards excessive humidity of the prior art structures, but modified in such a manner as to eliminate

2

the undesirable absorption in the blue region of the spectrum.

It is, therefore, the principal object of this invention to provide a cyan naphthol color former having a low absorption in the blue portion of the spectrum.

A further object is to provide naphthol coupler compounds which produce cyan dyes having a high degree of heat and light stability.

A still further object is to provide naphthol coupler compounds which produce cyan dyes having a high degree of resistance under conditions of high humidity.

Other objects will appear hereafter as the description proceeds.

The aforesaid objects are accomplished according to our invention by providing cyan coupler compounds formulistically depicted below:



wherein X is a mildly electropositive neutral substituent such as lower alkyl, i.e., methyl, ethyl, butyl, etc., halogen, e.g., chlorine, bromine, etc. and lower alkoxy, methoxyl, ethoxy propoxyl, butoxyl, etc. and R is an alkyl group of from 10 to 20 carbon atoms, e.g., decyl, undecyl, dodecyl, tridecyl, tetrade cetyl, pentadecyl, hexadecyl, heptadecyl, octadecyl, nonadecyl, etc.

Specific compounds forming within the ambit of the above formula include the following structures:

35



40



45



50



55



70



In general the couplers as described herein are prepared by reacting the phenyl ester of 1-hydroxy-2-naphthoic acid with the appropriate aniline, a condensation which is commonly referred to as the Salol condensation. The so-obtained couplers are then sulfonated in the 4-position using chlorosulfonic acid as the sulfonating agent.

The following examples are illustrative of the preparation of the couplers described herein but such examples are not to be taken as limiting or in any way construing the invention.

#### Preparation of Compound 3



1 - hydroxy - 5' - methyl-2'-tetradecoxy-4-sulfo-2-naphthoanilide was prepared as follows: 4.9 g. of 2'-tetradecoxy-5'-methyl-1-hydroxy-2-naphthoanilide was dissolved in 25 cc. of dry carbon tetrachloride to which 1 cc. of chlorosulfonic acid was added at room temperature with stirring. Stirring was continued for one hour at room temperature and for three hours under reflux. The mixture was allowed to cool to 20° C. and 1 g. of sodium chloride in 10 cc. of water was added with stirring. All the volatile material was removed under reduced pressure and the residue of the sodium salt of the coupler was crystallized from acetonitrile. Yield: 3.6 g. (60%) M.P. 104-105° C.

*Analysis.*—Calc.: N, 2.37; S, 5.41. Found: N, 2.50; S, 5.40.

1 - hydroxy - 5' - methyl-2'-tetradecoxy-2-naphthoanilide was prepared as follows: 11.1 g. of 3-amino-4-tetradecoxytoluene and 10.3 g. of phenyl-1-hydroxy-2-naphthoate was heated together to 140° C. and held there for two hours. The hot melt was poured into an evaporating dish and triturated with methanol. The solid was filtered off and crystallized from isopropanol. The yield of purified material was 9.2 g. (54%) M.P. 58-59° C.

*Analysis.*—Calc.: N, 2.85. Found: N, 3.01.

3-amino-4-tetradecoxytoluene was prepared as follows: 32 g. of 3-acetamino-4-tetradecoxyltoluene and 150 cc. of acetic acid and 115 cc. of concentrated HCl were refluxed

for three hours. After cooling to room temperature the solution was poured into an excess of cold water. The amine hydrochloride which separated was filtered off, washed with water and sucked dry. The solid was redispersed in water and 40 cc. of concentrated NH<sub>4</sub>OH was then added. After heating a short time on the steam bath the free base separated as an oil which, on cooling, solidified. It was filtered off, washed with water and crystallized from methanol. Yield: 23 g. (81%) M.P. 43-44° C.

*Analysis.*—Calc.: N, 4.39. Found: N, 4.45.

3-acetamino-4-tetradecoxyltoluene was prepared as follows: 23 g. of 3-acetamino-p-cresol, and 30 g. of tetradearyl bromide and 7.5 g. of sodium methoxide in 375 cc. of absolute alcohol was refluxed for six hours. The mixture was allowed to stand at room temperature overnight and then poured into an excess of water. The solid which separated was filtered, washed with water and crystallized from methanol. The yield of purified product was 29.8 g. (60%) M.P. 62-63° C.

*Analysis.*—Calc.: C, 76.40; H, 10.86; N, 3.87. Found: C, 76.00, 75.62; H, 10.88, 10.57; N, 4.16, 4.26.

The above-detailed synthesis of Compound 3 is generally applicable to the coupler compounds as described herein. For instance, Compound 5 can be prepared by reacting 1-hydroxy-2-naphthoic acid phenyl ester with 4-ethyl-2-tridecoxy aniline followed by sulfonation with chlorosulfonic acid. Compound 7 can be produced by condensing 1-hydroxy-2-naphthoic acid phenyl ester with 4-ethyl-2-deoxy aniline followed by sulfonation with chlorosulfonic acid. The remaining coupler compounds formulistically depicted elsewhere can be produced in like manner by condensing the appropriate long chain alkoxy aniline with the phenyl ester of 1-hydroxy-2-naphthoic acid. The requisite ortho long chain alkoxy aniline can be obtained by methods known in the organic chemical art, and the detailed preparation of these entities is not deemed necessary, since such knowledge would be obvious to a skilled organic technician.

It is to be noted that the salt forming sulfo group is attached to the 4 or coupling position of the color formers. However, the indoaniline dye images produced on color development do not contain the sulfo substituent since it is eliminated in the color-forming reaction. Thus, whereas the color formers are soluble in aqueous alkali or solutions thereof, the dyes themselves have no solubilizing group and are therefore of a lipophilic nature. This is a valuable property since it tends to make the dyes resistant to fading under conditions of excessive humidity.

Our color formers may be incorporated in silver halide emulsions in the manner known to the art. Thus, the couplers are dissolved in an aqueous alkaline solution and are then combined with the silver halide emulsion, which is then coated on a suitable support or base.

Although it is a common practice to incorporate our color formers in gelatin layers, other photographic colloids may also be employed for this purpose. Thus, synthetic resins such as polyvinyl alcohol, carboxymethyl cellulose, starch, gum arabic, casein, zein, etc. can be used as carriers.

The primary aromatic amino developing agents of the type used to produce colored photographic images with color couplers are known to the photographic field.

Suitable developing agents include the various alkyl phenylenediamines such as 4-aminoaniline, 4-ethylaminoaniline, 2-diethylaminoaniline, 4-dialkylaminoaniline, e.g., 4-dimethylaminoaniline, 4-diethylaminoaniline, 4-[N-( $\beta$ -hydroxyethyl)-N-ethyl]aminoaniline, 4-amino-N-ethyl-N-( $\beta$ -methanesulfonamidoethyl)-2-methylaniline sulfate and the like. The above developing agents are preferably used in the form of their salts such as the hydrochloride or hydrosulfate as they are more soluble and stable than the free bases. All of these compounds have a primary amino group which enables the oxidation product of the

developer to couple with the color compounds to form dye images. After removal of the silver image by bleaching and fixing in a manner well known in the art, the color image remains in the emulsion. A typical developing solution can be prepared as follows:

|                               | G.  | 10 |
|-------------------------------|-----|----|
| 2-amino-5-diethylaminotoluene | 2   |    |
| Sodium carbonate (anhydrous)  | 20  |    |
| Sodium sulfite (anhydrous)    | 2   |    |
| Potassium bromide             | 0.2 |    |
| Water to make 1 liter.        |     |    |

The exposed silver halide emulsions containing the color formers are developed in the above solution in the usual manner.

Bases which are useful for holding the emulsion layers containing our color couplers may be any of the usual supports. For instance, bases such as a cellulose ester, polystyrene, polyamide, polyester or a non-transparent reflecting material such as paper have proved suitable for this purpose.

As pointed out elsewhere, the cyan naphthol color formers produced in accordance with the invention yield on color development cyan dye images having a low absorption in the blue range of the electromagnetic spectrum. As a consequence, the images are not plagued with the undesirable greenish hues characteristic of the dye images of the prior art. This constitutes a decided advantage in reproducing an accurate rendition of the color aspects of a colored subject. In addition to these desirable spectral properties, our color formers display high stability when subjected to excessively high humidity and light intensities.

It is to be understood that the extent of our invention is not limited except as necessitated by the appended claims.

We claim:

1. A photographic silver halide emulsion containing as a color forming coupler a compound having the following formula:

5

15

20

25

30

35



wherein X is a substituent selected from the class consisting of lower alkyl, halogen and lower alkoxy and R is an alkyl group of from 10 to 20 carbon atoms.

2. A photographic silver halide emulsion containing as a color forming coupler a compound having the following formula:



#### References Cited in the file of this patent

##### UNITED STATES PATENTS

2,357,394 Frohlich et al. Sept. 5, 1944  
2,704,709 Sprung Mar. 22, 1955

##### FOREIGN PATENTS

1,036,053 Germany Aug. 7, 1958  
649,660 Great Britain Jan. 31, 1951